

O. E. JACOBS.

PROCESS FOR THE DRYING AND CURING OF LUMBER.

APPLICATION FILED SEPT. 15, 1916.

1,333,848.

Patented Mar. 16, 1920.



Inventor

OSCAR E. JACOBS

Witnesses

M. H. Glasgow.  
G. B. Thompson.

By *Chappell & Earl*

Attorneys

# UNITED STATES PATENT OFFICE.

OSCAR E. JACOBS, OF KALAMAZOO, MICHIGAN.

## PROCESS FOR THE DRYING AND CURING OF LUMBER.

1,333,848.

Specification of Letters Patent. Patented Mar. 16, 1920.

Application filed September 15, 1916. Serial No. 120,893.

To all whom it may concern:

Be it known that I, OSCAR E. JACOBS, a citizen of the United States, residing at the city and county of Kalamazoo, State of Michigan, have invented certain new and useful Improvements in Processes for the Drying and Curing of Lumber, of which the following is a specification.

This invention relates to an improved process for the drying and curing of lumber.

The object of this invention is to eliminate all moisture from the lumber without injuring the texture or quality of the same in any way.

I accomplish the object of my invention by the process described in the following specification. The invention is clearly defined and pointed out in the claims.

My process may be carried out in an apparatus similar to that illustrated in U. S. Patent No. 217,002, issued July 1, 1879, to L. S. Robbins, for process or apparatus for treating wood or lumber; or in an apparatus comparable to that appearing in U. S. Patent No. 1,186,555, issued June 13, 1916, to Derby and Dargie, for process for the treatment of wood. The details of construction of such apparatus, however, are not material and can be greatly modified.

I illustrate an apparatus adapted to carry out my invention, it being an apparatus that may be made use of for various purposes, and my invention may be carried out in any suitable apparatus, this being illustrated merely as an effective apparatus for the purpose.

The apparatus illustrated comprises a steam chamber or kiln 1 in which there is a track 2 for receiving a truck 3 with a load of lumber or timber 4 which is piled with suitable spaces 5 between it. The kiln door 6 is provided with a gasket 7 for hermetically closing the same. A steam pipe 8 controlled by the valve 9 delivers steam to the chamber or kiln and the exhaust pipe 10 connects to a vacuum pump 11 for discharging the vapor and air from the inside of the kiln outwardly through the pipe 12. The pump 11 is operated through the piston rod 13 and eccentric 14 carried upon shaft 15 driven by the tight and loose pulley 16. A steam pipe 17 delivers to a coil 18 within the kiln the circulation discharge 19 extending out through the wall of the kiln. Pipe 20 is for exhausting the steam after the pressure treatment. This provides a

suitable apparatus for carrying out the steps of my improved process.

The first step of my improved process is to inclose the lumber in a suitable cylinder or retort which can be closed air tight, within which is disposed a steam coil for heating the same. I heat the lumber to temperature of about 100° F. for 20 or 30 minutes by means of the steam coils until the surface of the lumber is air dry and fairly warm.

For the second step, I introduce live steam at a temperature below 250° F., preferably at a pressure of about 20 pounds to the square inch, and maintain the same for about 20 minutes for the treatment of lumber about one inch in thickness. I have found that a temperature of above 250° F. is likely to injure the quality of wood fiber.

For the third step, after the wood has thus become thoroughly saturated with the hot steam, I blow off the steam, which takes a period of 2 or 3 minutes and then connect a vacuum pump and produce a vacuum of from 20 to 28 inches, keeping the pump in operation to carry off the moisture as it expands into vapor from the wood. From this treatment, it will be very clear that there is little or no air in the cylinder or retort when the steam is blown off and the vacuum is created by the drawing off of the vapor itself. I endeavor to keep the temperature of the wood within the retort in the early stage of the evaporation substantially at or above the boiling point within the vacuum chamber. To do this, I turn on the steam in the coils that were used for heating in the first place and then maintain the temperature at about 100° to 120° F. so that the moisture in the wood will be very rapidly evaporated. Of course, it is not possible to materially heat the wood after the vacuum is created, but I find that it is possible by the use of the coils to substantially maintain the temperature at about 100° F. I maintain the temperature a little higher, about 120°, at the finish. I maintain the vacuum as near as may be for a period of from 16 to 18 hours for one inch stock; for three-eighths inch stock about 7 hours of time is sufficient; for four-by-four stock 17 hours has been found to be sufficient to extract all the moisture. When the moisture has been extracted the lumber has become thoroughly dried and can be removed.

75

80

85

90

95

100

105

110

This process avoids any checking of the wood and dries the same apparently from the inside out so that the entire fiber of the lumber that is subjected to the whole treatment is equally dried and there is no checking or splitting or any undue hardening of the surfact or of any part of the lumber that has been submitted to the treatment.

Having thus described my invention, what I claim as new and desire to secure by Letters Patent, is:

1. The process of treating lumber consisting of inclosing the same in a suitable retort and heating the same to about 100° F. for a period sufficient to thoroughly air dry the surface of the same then subjecting the same to live steam at about 20 pounds pressure and not to exceed 250° heat until the entire substance of the lumber has become evenly heated, thereupon blowing off steam and subjecting the chamber to a vacuum action and maintaining heat within the vacu-

um and continuing the vacuum action with the lumber at a temperature of about 100° to 120° F. until the same is dried.

25

2. The process of treating lumber consisting of inclosing the same in a suitable retort and heating the same to about 100° F. for a period sufficient to thoroughly air dry the surface of the same then subjecting the same to live steam at about 20 pounds pressure and not to exceed 250° heat until the entire substance of the lumber has become evenly heated, thereupon blowing off steam and subjecting the chamber to a vacuum action 30 until the same is dried.

30

In witness whereof, I have hereunto set my hand and seal in the presence of two witnesses.

OSCAR E. JACOBS. [L. s.]

Witnesses:

THOMAS W. BARLOW,  
R. M. DANFORTH.